

## UNITED STATES PATENT OFFICE

2,029,310

## FELT AND PROCESS OF MAKING SAME

Pierre Drewsen, Sandusky, Ohio, assignor to The  
Barrett Company, a corporation of New Jersey

No Drawing. Application February 4, 1926, Serial  
No. 86,098. Renewed January 27, 1934

33 Claims. (Cl. 92—3)

This invention relates to the production of paper or felt. It relates particularly to processes of producing felt, suitable for saturation with tar, asphalt or other saturants or waterproofing materials, which may be used, for example, for building, sheathing, roofing or other purposes.

Heretofore the manufacture of saturating felt has been accomplished by the utilization of one or more of the following materials: #1 rags, which contain substantially a mixture of cotton and wool; #2 rags, which contain substantially cotton; #3 rags, which contain jute fiber in the form of waste bagging; #4 rags, which contain substantially old carpets, composed largely of jute, with quantities of cotton and wool; #5 rags, which contain rag clippings of all grades with varying amounts of paper; and paper stock, composed largely of waste paper. These materials are partially disintegrated in rag cutters and, thereafter, while in suspension in water, are beaten in paper mill beaters, then jordanized if desired and finally formed into a continuous sheet of paper on Fourdrinier or cylinder paper machines.

My invention contemplates the treatment of cereal and other annual crop fibers and other vegetable fibers in such a manner as to produce fibers of three classes, to wit: (1) fibers in which strength is the predominating characteristic; (2) fibers of high absorptive capacity; (3) filler fibers relatively low in saturating capacity and strength. My invention further contemplates the blending of two or more of these three classes of fibers in such a manner, as is hereinafter more fully described, as to produce a sheet of felt having the requisite strength and absorptive capacity for the purpose for which it is intended to be used.

All unsized and moderately well beaten fibers which will run on a paper-making machine and form a sheet of paper have some strength and some saturating capacity, it being usually the case, however, that as the comparative strength of a fiber is increased as, for instance, by prolonged beating, the comparative saturating capacity thereof is diminished. The amount of saturant which felt paper will absorb, besides depending upon the absorptive capacity of the sheet, depends upon the condition of saturation—such as time of immersion of the sheet, temperature of the saturant and pressure of the squeeze rolls, and the quality of the saturant—such as composition and viscosity thereof. There are many grades of saturating felt, some manufactured to absorb a relatively small amount of sat-

urant as, for instance, tar saturated felts containing 85%, or less, of saturant based on the dry weight of the felt; while some are produced for the manufacture of composition shingles, the percentage of asphalt absorbed sometimes exceeding 200%. In general, therefore, where felts of all kinds, both slightly and highly absorbent, are made it is desirable to have strength-giving fibers, good saturant carrying fibers and fibers to control saturating qualities.

Of these three classes of fibers, those to be used principally for imparting the element of strength to a sheet of saturating felt may be prepared as follows: Jute, that is waste bagging otherwise called #3 rags, is cooked by the calcium pentasulphide process, substantially as described in U. S. Patent No. 996,225, to Viggo Drewsen granted June 27, 1911 is then washed until free from spent cooking liquors and afterward defibered in a beating engine. The fiber thus produced has been found to be greatly different in character from the uncooked bagging or jute as known to the prior art. Polysulphides of certain other alkali or alkali earth metals may be used instead of calcium pentasulphide with similar results. Good results have also been obtained in producing a strength fiber by cooking raw jute or jute bagging, at an elevated temperature of from 130° to 150° C., in a solution of sodium carbonate containing about 10% by weight of sodium carbonate based on the weight of the raw fiber being cooked. It may be desirable to use a 10% solution of lime instead of the sodium carbonate solution.

Flax tow, made from American or Canadian flax straw by the well known breaking process, by which the shive or interior woody portion is largely removed, has been found to also give a very useful strength fiber when treated in a manner similar to that above set forth.

It has also been found that a strength fiber may be produced from jute or flax tow by treating same in the ordinary type of beating engine with water at 90° to 100° C., to which approximately 10% more or less of alkali, such as caustic soda, caustic lime, etc., based upon the dry weight of the fiber to be treated, has been added. The fiber, of course, should be thoroughly washed with water before it is used as a component in the felt.

It has also been found that unbleached sulphite or kraft pulp may be used successfully as a strength fiber in my formulae for producing felt.

Of these three classes of fibers, those to be used principally for imparting high absorptive

capacity to a sheet of saturating felt may be prepared as follows: Spruce or hemlock, chips or shavings may be cooked by the above calcium pentasulphide process or by the sodium pentasulphide process, after which the fibers are disintegrated by treatment with edge runners or in the ordinary form of beating engine or jordan engine. Wood substances may also be treated at elevated temperatures of 90° to 100° C. in the ordinary type of beating engine in a solution of caustic soda or similarly acting alkali, the amount of alkali in the solution being equal to more than 10% of the dry weight of the wood substances, after which the fibrous substance is washed and disintegrated in a beating engine. Absorptive fibers may also be produced by treating wheat straw, rye straw, oat straw, rice straw or barley straw or other cereal or annual crop fiber in a digester with water at elevated temperatures, for instance, from 120° to 150° C., for a short period of time sufficient only to thoroughly soak the fibrous material, which material is then disintegrated in the ordinary type of beating engine. This type of fiber may also be produced from the same raw materials by beating said fibers at lower temperatures, such for instance as 90°-100° C. When beating such materials at about 50° C. it has been found more satisfactory to add about 10% sodium carbonate. When beating such materials at atmospheric temperature, sodium carbonate may be replaced by caustic soda, altho such substitution tends to increase the rapidity of the treatment. The use of too strong a chemical solution for too long a time, is to be avoided, since too extended a treatment will cut down the absorptivity of the fiber.

When cotton hull fiber, namely minute seed hairs obtained from cotton seed hulls after the removal of the cotton and cotton linters, containing a substantial proportion of hull particles, is cooked by the calcium or sodium pentasulphide process, substantially as described previously for jute or flax tow, the hull particles become softened to such an extent that they yield readily to the action of a beater or other fiber disintegrating engine and form a very good absorptive fiber.

Of these three classes of fibers, those to be used principally for filler fibers may be prepared as follows: Cereal or other crop fibers, such as wheat straw, rye straw, oat straw, rice straw, barley straw and others when thoroughly cooked by the calcium or sodium pentasulphide process and washed to free the cooked fiber from spent alkaline liquors, may be reduced in a beating or defibering engine. These same raw materials may also be cooked at an elevated temperature and pressure in sodium carbonate, caustic soda or other alkali of moderate percentage and afterwards washed and beaten, or they may be cooked and beaten in a beating engine at 90°-100° C. in the presence of a 10% solution of caustic soda, i. e. a solution containing caustic soda in amount equal to 10% of the weight of the straw. When so treated such fibers are low in strength and saturating capacity and, therefore, may be used as filler fibers.

Thus I have described various processes for producing each of the three types of fibers, any number of which I may employ. Depending upon the type of felt desired to be produced, and the matter incorporated therein, various percentages of each or various percentages of only two of the three types may be employed. For instance,

if a sheet of high strength is desired and high absorptive capacity is not necessary, strength and filler fibers alone may be combined. If a sheet of high absorptive capacity is desired, strength and absorptive fibers alone may be combined. If an average sheet is desired all three types of fibers may be combined, the filler fiber being added, because usually of low cost, to bring up the weight of the sheet.

For some kinds of building paper I find it quite satisfactory to use a felt furnish of approximately 15% cooked jute fiber or cooked flax tow or other cooked strength fiber and 85% well cooked cereal crop fiber which, altho moderately non-absorptive, nevertheless, has sufficient absorptive capacity to give, together with the strength ingredient, a sheet which will absorb approximately 100% of tar. In a similar manner, to make a shingle felt for high asphalt saturation, I may employ approximately 25% of cooked jute, flax tow, sulphite or kraft pulp, approximately 40% absorbent cereal or other crop or vegetable fiber and approximately 35% of well cooked crop fiber, the latter acting as a filler for controlling the saturating quality of the sheet. A sheet thus produced may have a saturating capacity of as high as 200% based upon the dry weight of the felt being saturated. Any one or more of the above may be used in the same felt furnish or one or more of them may be used in connection with the old type of rag furnish as a substitute for all or part of any one class of raw prepared rags or fibers.

In other words, my invention contemplates the matter of accurate control during the production of the felt. If a sheet of great strength is desired a greater percentage of strength fiber should be added. If a sheet of high absorptive capacity is desired a greater percentage of the class of absorptive fibers should be added to the felt furnish. The quality of the finished product is bound to vary from time to time because of irregularity of raw materials and it is contemplated by this invention to regulate the finished product by slightly increasing or decreasing the constituents of the furnish, such as adding or subtracting from the percentage of filler fibers used, or increasing or decreasing the amount of absorptive fibers employed.

Among the advantages of my invention are that inexpensive raw materials are employed, which materially reduces the cost of the finished product, the conversion of these raw materials into fibers of the proper quality is readily accomplished, a felt of any desired quality may easily be obtained and the uniformity of any particular type of felt can be easily maintained during its manufacture.

I claim:

1. The process of producing roofing felt which comprises cooking jute fibers to produce fibers which when incorporated in the felt impart strength thereto, separately cooking vegetable fibers to produce absorptive fibers, separately cooking cereal fibers under conditions of increased severity as compared with the treatment of the said vegetable fibers, and admixing the three types of fibers thus produced in the proportion of from approximately 15 to approximately 25 per cent of strength fibers, approximately 40 to approximately 85 per cent of absorptive fibers, and the remainder cooked cereal fibers to produce a felt sheet having the desired strength and absorptive characteristics.
2. The method of producing roofing felt which

comprises beating jute fibers in an alkaline solution to produce fibers which when incorporated in the felt impart strength thereto, beating straw fibers to produce absorptive fibers, beating cereal fibers under conditions of increased severity as compared with the treatment of the said straw fibers to produce filler fibers, and blending the three types of fibers in desired proportions to produce a felt sheet having the desired strength and absorptive characteristics.

3. The process of producing felt which comprises cooking jute fibers to produce fibers imparting strength to the sheet in which they are incorporated, beating vegetable fibers to produce fibers imparting high absorptive characteristics to the sheet in which they are incorporated, beating cereal fibers under conditions of increased severity as compared with the treatment of the said vegetable fibers to produce filler fibers, and blending the three types of fibers in desired proportions to produce a felt sheet having the desired strength and absorptive characteristics.

4. The process of producing felt which comprises beating jute fibers to produce fibers imparting strength to the sheet in which they are incorporated, cooking vegetable fibers to produce fibers imparting high absorptive characteristics to the sheet in which they are incorporated, beating cereal fibers under conditions of increased severity as compared with the treatment of the said vegetable fibers to produce filler fibers, and blending the three types of fibers in desired proportions to produce a felt sheet having the desired strength and absorptive characteristics.

5. The process of producing felt which comprises beating jute fibers to produce fibers imparting strength to the sheet in which they are incorporated, cooking vegetable fibers to produce fibers imparting high absorptive characteristics to the sheet in which they are incorporated, cooking cereal fibers under conditions of increased severity as compared with the treatment of the said vegetable fibers to produce filler fibers, and blending the three types of fibers in desired proportions to produce a felt sheet having the desired strength and absorptive characteristics.

6. The process of producing felt which comprises treating jute fibers in an alkaline solution to produce fibers which when incorporated in the felt impart strength thereto, treating straw in water at an elevated temperature to produce absorptive fibers, and blending the resultant fibers to produce a felt sheet having the desired strength and absorptive characteristics.

7. A roofing felt comprising jute fibers beaten in an alkaline solution, said fibers imparting strength to said felt, straw fibers beaten to produce absorptive fibers, and filler fibers formed by beating cereal fibers under conditions of increased severity as compared with the treatment of said straw fibers, said three types of fibers being blended to produce a felt having the desired strength and absorptive characteristics.

8. A roofing felt comprising jute fibers beaten to produce fibers imparting strength to said felt, vegetable fibers cooked to produce fibers imparting high absorptive characteristics to said felt and cereal fibers beaten under conditions of increased severity as compared with treatment of said vegetable fibers to produce filler fibers, said three types of fibers being blended in desired proportions to produce a sheet having the desired strength and absorptive characteristics.

9. A roofing felt containing jute fibers which have been treated in an alkaline solution to pro-

duce fibers which impart strength to said felt, absorptive fibers produced by treating straw in water at an elevated temperature, said fibers being blended to produce a felt sheet having the desired strength and absorptive characteristics.

10. As an article of manufacture, a roofing felt consisting of jute fibers imparting strength to the felt, straw fibers having the characteristics of incompletely disintegrating straw which imparts high absorptive characteristics to the felt, and cereal fibers having the characteristics of cereal straw more completely disintegrated than the aforementioned straw fibers.

11. As an article of manufacture, felt consisting of from approximately 15 to approximately 25 per cent jute fibers, approximately 40 to approximately 85 per cent straw fibers having the characteristics of incompletely disintegrated straw which impart high absorptive characteristics to the felt, and the remainder cereal fibers having the characteristics of cereal straw more completely disintegrated than the aforementioned straw fibers.

12. The process of producing felt paper which comprises blending jute fibers which have been cooked by the pentasulfide process with felt paper making material that will give high saturating qualities to a sheet and forming a sheet of felt paper containing said components.

13. The process of producing felt paper which comprises making a pulp containing jute cooked by the pentasulfide process and substantially resolved into its ultimate fibers, said fibers possessing only a moderately absorptive quality for waterproofing saturants and forming a sheet from said pulp.

14. As an article of manufacture, a felt paper consisting of vegetable fibers cooked in such a manner that their original strength remains substantially unchanged, material that imparts high saturating qualities to the paper and a filler fiber of only moderately absorptive quality made by cooking straw in an alkaline polysulfide solution.

15. As an article of manufacture a felt paper consisting of 15% to 25% of jute which has been cooked by the pentasulfide process, 40% to 85% of crop fibre which has been cooked partially to such an extent as to give high saturating qualities to the sheet and 35% or less of vegetable crop fibre which has been thoroughly cooked to impart high strength quality thereto, substantially as described.

16. As an article of manufacture, a felt paper consisting of 25% cooked jute, 40% cooked absorptive fiber from a straw, and 25% well cooked filler fiber from a straw.

17. A process for the production of a felt paper which comprises cooking jute in an alkaline medium, cooking a straw in the presence of water for a period of time sufficient only to thoroughly soak the straw, thoroughly cooking a straw in an alkaline medium until a fiber possessing little strength is obtained, and then blending the resultant fibers, pulping the blended mixture of fibers, and sheeting the pulped mass.

18. A process for the production of a felt paper which comprises cooking jute in an alkaline medium at a temperature of from about 90° to 150° C., cooking a straw in an alkaline medium at a temperature from about 90° to 100° C., thoroughly cooking a straw in an alkaline medium until a fiber possessing little strength is obtained, and then blending the resultant fibers, pulping the blended mixture of fibers, and sheeting the pulped mass.

19. A process for the production of a felt paper which comprises cooking a straw in the presence of a polysulfide to form a strength fiber, an absorptive fiber, and a filler fiber, blending the fibers so obtained, making a pulp of said blended fibers and forming a sheet therefrom.
20. A bitumen-saturated felt adapted for use in the manufacture of felt base roofing, comprising strength, absorptive, and filler fibers, the strength fibers being selected from the group: (a) cooked jute fibers, (b) beaten jute fibers, and (c) wood fibers converted into strength fibers by chemical treatment under conditions of increased severity as compared with the treatment of the wood fibers converted into absorptive fibers, the absorptive fibers being selected from the group: (1) wood fibers converted into absorptive fibers by chemical treatment and (2) annual vegetable crop fibers, and the filler fibers being constituted of annual vegetable crop fibers treated under conditions of increased severity as compared with the treatment of the annual vegetable crop fibers constituting the absorptive fibers.
21. A bitumen-saturated felt adapted for use in the manufacture of felt base roofing, comprising strength and absorptive fibers, the strength fibers being selected from the group: (a) cooked jute fibers, (b) beaten jute fibers, and (c) wood fibers converted into strength fibers by chemical treatment under conditions of increased severity as compared with the treatment of the wood fibers converted into absorptive fibers, the absorptive fibers being selected from the group: (1) wood fibers converted into absorptive fibers by chemical treatment and (2) annual vegetable crop fibers.
22. Bitumen-saturated felt adapted for use in the manufacture of felt base roofing comprising strength and absorptive fibers, both of said fibers being produced by chemical treatment of wood fibers as such and as distinguished from the treatment of paper or rags; the wood fibers converted into strength fibers being treated under conditions of increased severity as compared with the treatment of the wood fibers converted into absorptive fibers, said saturated felt sheet containing bituminous saturant in an amount equal to at least 200 per cent of the dry weight of the felt.
23. A bitumen-saturated felt as defined in claim 22 in which the strength fibers are selected from the group: sulphite pulp and kraft pulp.
24. A bitumen-saturated felt as defined in claim 22 in which the absorptive fibers comprise wood fibers cooked in an aqueous alkaline medium at an elevated temperature, said medium containing at least one reagent from the group: alkali metal hydroxides, alkali metal polysulfides, and alkali earth metal polysulfides.
25. Bitumen-saturated felt as defined in claim 22 and containing in addition to the strength and absorptive fibers filler fibers prepared from annual crop fibers.
26. Bitumen-saturated felt adapted for use in the manufacture of felt base roofing comprising strength and absorptive fibers, the strength fibers being produced by pulping of wood fibers as such and as distinguished from the treatment of paper or rags and the absorptive fibers being produced by the mechanical disintegration of annual crop fibers in an aqueous medium, said saturated felt sheet containing bituminous saturant in an amount equal to at least 200 per cent of the dry weight of the felt.
27. A felt sheet adapted to be saturated with waterproofing material and comprising strength fibers from the group: sulphite pulp and kraft pulp, and absorptive fibers prepared by disintegrating fibers of vegetable origin in an aqueous medium so as to increase their absorptive capacity, the absorptive fibers being blended with the strength fibers after disintegration of the absorptive fibers and before sheeting the resultant mixture.
28. A felt sheet adapted to be saturated with a bituminous waterproofing saturant and comprising strength fibers from the group: sulphite pulp and kraft pulp, and at least about 40 per cent based on the dry weight of the unsaturated felt absorptive fibers prepared by disintegrating vegetable fibers in an aqueous medium so as to increase their absorptive capacity, said felt being capable of absorbing at least 200 per cent of its dry weight of bituminous saturant.
29. A felt sheet adapted to be saturated with bituminous material for use in the manufacture of felt base roofing consisting entirely of wood fibers and annual crop fibers.
30. A process for producing felt which comprises treating wood with a solution of caustic soda, the amount of caustic soda employed being at least 10 per cent of the weight of the wood, at temperatures of not less than 90° C. to produce fibers of high absorptive capacity, mixing said fibers with other fibers and forming the mixture into a felt sheet of high absorptive capacity.
31. A process as claimed in claim 30 in which the said other fibers are of greater strength but less absorptive capacity than said absorptive wood fibers.
32. A process of producing felt which comprises treating wood with a solution of caustic soda at a temperature of not less than 90° C. to produce fibers of open structure and high absorptivity, mixing said fibers with other fibers and forming the resultant mixture of fibers into a felt sheet.
33. A waterproof felt sheet comprising a substantial proportion of wood fibers of high absorptive capacity produced by treating wood substances with a solution of caustic alkali at temperatures higher than 90° C.; and other fibers, said felt being impregnated with a waterproofing saturant.

PIERRE DREWSSEN.

CERTIFICATE OF CORRECTION.

Patent No. 2,029,310.

February 4, 1936.

PIERRE DREWSSEN.

It is hereby certified that error appears in the printed specification of the above numbered patent requiring correction as follows: Page 3, second column, line 9, claim 10, for "disintegrating" read disintegrated; line 55, claim 16, for "25%" read 35%; and that the said Letters Patent should be read with these corrections therein that the same may conform to the record of the case in the Patent Office.

Signed and sealed this 3rd day of March, A. D. 1936.

Leslie Frazer

Acting Commissioner of Patents.

(Seal)